

## UNITED STATES PATENT OFFICE

2,008,282

CHROMIUM PLATED ARTICLE AND METHOD  
OF MAKING THE SAME

William H. Keen, Albany, N. Y.

No Drawing. Application March 31, 1932,  
Serial No. 602,384

3 Claims. (Cl. 76—104)

The present invention relates to chromium plated articles and has as an object to provide a corrosion resisting product of good quality, which will be commercially satisfactory and possible of manufacture at low cost.

The invention has been evolved in connection with the development of cutlery and such an embodiment will be more particularly described for the purposes of disclosure of the principles 10 of the invention, but it will be understood that the description is illustrative merely and not intended as defining the limits of the invention.

Cutlery made of the best quality of corrosion resisting high chromium steel has become extremely popular during the last several years, but the cost of the steel limits its use to a field in which the requirement of quality is primary. In order to meet the demand for low price cutlery, attempts have been made to provide a less 20 expensive article by chromium plating other steels, such as carbon steel. Knives of this manufacture, however, have been unsatisfactory in use for the reason that when the chromium plate is disturbed, either by the wear due to use or by 25 the sharpening of the knife, the exposed steel stains and corrodes. The result has been that the manufacture of knives of this type has been abandoned as not producing a commercially satisfactory article.

The present invention provides an improved article which is made of a corrosion resisting steel chromium plated. The steel offers sufficient resistance to corrosion so that when exposed by the removal of the chromium plate it will still present a satisfactory appearance. The quality of 35 the steel, furthermore, is such that a satisfactory sharp edge can be maintained on knives.

Cutlery produced in accordance with the present invention has the further advantage that the chromium plate is hard and resistant to scratches. In fact, in this particular regard it is superior to commercial stainless steel cutlery. It possesses a finish which is noticeably superior in appearance to the ordinary glaze and nearly equal to the 45 popular "mirror" finish.

The composition of the steel alloy should be so selected as to provide a reasonable resistance to corrosion under the conditions of use when exposed by the partial removal of the chromium plate and it should be of a quality to maintain a satisfactory edge, in the case of knives, in order to meet commercial requirements. At the same time the composition should be one which can be manufactured at a relatively low cost. A steel

meeting these requirements may contain, for example, approximately,—

|           | Per cent      |   |
|-----------|---------------|---|
| Carbon    | 0.05 to 1.20  |   |
| Chromium  | 5.00 to 12.00 | 5 |
| Silicon   | 0.00 to 0.50  |   |
| Manganese | 0.20 to 0.80  |   |

with the remainder principally iron.

There are certain advantages in adding a small 10 amount of magnesium, as, for example, 0.10 to 2.50%.

It will be understood that other elements such as are ordinarily found in steel either as impurities or as desirable components may be present in this steel, in the event that corresponding properties are desired or a less expensive product is preferred. Such steels may contain, for example, nickel, vanadium, molybdenum, tungsten or other elements required to produce characteristic properties that may be desired. 15 20

A preferred steel providing knives of good quality may contain approximately—

|           | Per cent     |    |
|-----------|--------------|----|
| Carbon    | 0.30 to 0.40 | 25 |
| Chromium  | 7. to 9.     |    |
| Magnesium | 0.20 to 0.40 |    |
| Silicon   | 0.10 to 0.30 |    |
| Manganese | 0.25 to 0.45 |    |

Steels of the compositions above indicated can 30 readily be forged or rolled and can be produced at about half the cost of steels made according to the usually accepted requirements for good quality corrosion resisting steels.

Knives are preferably hardened and tempered before plating. This applies also to other articles, though perhaps with less force, the treatment adding to the corrosion resistance. The 35 hardening treatment may, of course, be varied somewhat but if the steel is of the preferred composition above indicated it may be suitably hardened by first heating to a temperature of 1800° F. and quenching in oil thus producing a martensitic quality in the steel.

If it is desired to use a hard rolled steel and 45 avoid the hardening and tempering operation, this may be done although somewhat at the expense of corrosion resistance. For such working a lower carbon content as from 0.05 to 0.25% is preferable thus providing a still less expensive 50 product and one which will still have commercially acceptable corrosion resistance.

Although the foregoing description relates to 55 chromium plated cutlery, it will be understood that other plating material such as silver, cad-

mium, tin or nickel can be substituted and the broader features of the invention can be applied to other articles such as automobile parts including bumpers, fenders and the like and even 5 to roofing without exceeding the scope of the invention as defined in the appended claims.

I claim—

- 10 1. A corrosion resisting article fabricated from a steel containing approximately 0.30 to 0.10% carbon, 5 to 9% chromium and 0.20 to 0.40% magnesium with the remainder principally iron, said article being plated with a metal of the group consisting of chromium, silver, cadmium, tin and nickel, said plating being molecularly in the same 15 condition as when first applied.
2. A corrosion resisting knife fabricated from

steel containing approximately 0.05 to 0.40% carbon, 5 to 9% chromium and 0.2 to 2% magnesium with the remainder principally iron, said knife being in hardened condition as the result of heating and quenching and having a chromium plate surface which plate is molecularly in the same condition as when first applied.

5 10 15 3. The method of producing a knife which comprises fabricating the knife of a corrosion resisting steel containing approximately 0.05 to 0.4% carbon, 7 to 9% chromium, 0.2 to 0.4% magnesium with the remainder principally iron, hardening the same and thereafter plating it with chromium.

WILLIAM H. KEEN. 15